# EUROPEAN PATENT SPECIFICATION

(11) **EP 3 433 021 B1**
(45) Date of publication and mention of the grant of the patent: **15.06.2022**
(21) Application number: 17711222.4
(22) Date of filing: 20.03.2017
(51) Int. Cl.: B03D 1/008, B03D 1/01, B03D 1/004, B03D 1/012

(54) **USE OF EMULSIFIER IN COLLECTOR COMPOSITION**
VERWENDUNG VON EMULGATOREN IN EINER SAMMLERMISCHUNG
UTILISATION D'ÉMULSIFIANTS EN COMPOSITION COLLECTRICE

(30) Priority: 22.03.2016 EP 16161733
(43) Date of publication of application: 30.01.2019
(73) Proprietor: Nouryon Chemicals International B.V., 6824BM Arnhem (NL)
(72) Inventor: NORDBERG, Henrik, 444 53 Stenungsund (SE); SMOLKO-SCHVARZMAYR, Natalija, 471 72 Hjälteby (SE); SVENSSON, Magnus, 444 46 Stenungsund (SE)
(74) Representative: LKGlobal UK Ltd.
(86) International application number: PCT/EP2017/056516
(87) International publication number: WO 2017/162563

(56) References cited:
- EP-A1- 0 687 726
- EP-A1- 2 650 352
- WO-A1-00/50560
- WO-A1-97/48850
- WO-A1-2005/113687
- US-A- 4 358 368
- Shell: "NEODOL 25-3 PRIMARY ALCOHOL ETHOXYLATE V2634 DERIVATIVES DATASHEET", , 1 October 2005 (2005-10-01), XP055307373, Retrieved from the Internet: URL:https://www.shell.com/content/dam/shel l/static/chemicals/downloads/products-serv ices/datasheet-neodol253.pdf [retrieved on 2016-10-04]
- Shell: "Objective Branching and Carbon Number Type in Detergent Range Alcohols* Branching and Carbon Number Type in Detergent Range Alcohols* Process Technology 2-Alkyl Total Carbon Branching (%) Branching** No. Type", , 16 September 2009 (2009-09-16), XP055307370, Retrieved from the Internet: URL:http://www.shell.com/business-customer s/chemicals/our-products/higher-olefins-an d-derivatives/neodol-alcohols-and-ethoxyla tes/_jcr_content/par/tabbedcontent/tab_178 0231844/textimage.stream/1447772619332/4a4 cf11b2dc70295885172e82b234a50b086e2e2e66c5 0387d73d6ffd4315f5e/neo06-qrc-alc-branchca rbonnum.pd [retrieved on 2016-10-04]
- Shell: "Typical distributions of NEODOL(TM) ethoxylate adducts", , 5 November 2009 (2009-11-05), XP055307376, Retrieved from the Internet: URL:http://www.shell.com/content/dam/shell /static/chemicals/downloads/products-servi ces/typical-distributionsneodolethoxylatea dducts.pdf [retrieved on 2016-10-04]
- Sasol: "Isotridecanol Ethoxylates MARLIPAL O13", Sasol Olefins & Surfactants, 31 December 2004 (2004-12-31), XP055307739, Retrieved from the Internet: URL:http://www.sasoltechdata.com/tds/marli pal.pdf [retrieved on 2016-10-05]
- Shell: "NEODOL 1", , 31 October 2005 (2005-10-31), XP055413830, Retrieved from the Internet: URL:http://www.shell.com/business-customer s/chemicals/our-products/higher-olefins-an d-derivatives/neodol-alcohols-and-ethoxyla tes/_jcr_content/par/tabbedcontent/tab_151 8891852/textimage.stream/1447832558700/06b 1039733643e2f2652a7e9615364f012f49cfce7c41 de605ff3305bfd0e05b/datasheet-neodol1.pdf [retrieved on 2017-10-09]
- Basf: "Lutensol Types, Technical Information", , 28 February 1997 (1997-02-28), XP055305778, Retrieved from the Internet: URL:http://www.timing-ouhan.com/images/lut ensoltotypes_.pdf [retrieved on 2016-09-27]
- Shell: "NEODOL 45-7 Primary Alcohol Ethoxylate", , 1 October 2005 (2005-10-01), XP055414581, Retrieved from the Internet: URL:http://www.shell.com/business-customer s/chemicals/our-products/higher-olefins-an d-derivatives/neodol-alcohols-and-ethoxyla tes/_jcr_content/par/tabbedcontent/tab_151 8891852/textimage_1790601121.stream/144783 5893901/3ecfb04481b694d6680b21d4b734ecd4ac ce4815e97e2fc9fa5da2c972046e48/datasheet-n eodol457.p [retrieved on 2017-10-11]

## Description

### Field of Invention

The present invention relates to the use of emulsifiers in branched alcohol alkoxylate-containing secondary collector compositions and the use of such compositions for the froth flotation of non-sulfidic ores, especially phosphate ores, in combination with a primary collector which is an anionic or an amphoteric surface active-compound.

### Background of the invention

Phosphate rocks contain calcium phosphate minerals largely in the form of apatite, usually together with other minerals, e.g. silicate minerals and carbonate minerals, such as calcite. Apatite is a generic name for a group of calcium phosphate minerals also containing other elements or radicals, such as fluorapatite, chlorapatite, hydroxylapatite, carbonate-rich fluorapatite and carbonate-rich hydroxylapatite.

It is well-known to separate the valuable phosphate minerals from the gangue by using a froth flotation process where the phosphate minerals are enriched in the float.

Good performance in a froth flotation process is achieved by a combination of, on the one hand, a good separation of the valuable mineral from the gangue by using a selective collector and, on the other hand, the froth characteristics. The froth characteristics include both the amount and the stability of the froth. It is important in the flotation process that the froth collapses as soon as possible after it leaves the flotation cell for the next step in the beneficiation process. A too stable froth will cause both entrainment of particles and froth product pumping problems. Entrainment, especially on a large scale, will result in decreased selectivity (grade, recovery). Problems with froth product pumping will make a process of flotation technically impossible.

Collector performance may be improved by using collector combinations of a primary (main) collector and a secondary collector (co-collector). In this document the term "collector composition" shall be used to describe compositions containing both a primary and a secondary collector.

For many decades secondary collectors have been used together with primary ionic collectors in salt-type mineral flotation to improve the performance of the primary collector. Nonylphenol ethoxylates have been the dominating nonionic surfactant used as a co-collector in a combination with sarcosine-type primary collectors in selective flotation of apatite from calcite-containing ores.

US 4,814,070 discloses the flotation of non-sulfidic ores wherein alkyl sulfosuccinates based on propoxylated and ethoxylated C8-C22 fatty alcohols are employed as a collector. However, nowhere in this document are fatty alcohols having a high degree of branching mentioned nor is it disclosed or suggested that they can be used without the sulfosuccinate function.

US 4,789,466 discloses the flotation of apatite ores with a collector composition that contains two components, wherein one is an ethoxylated and propoxylated fatty alcohol and the other is a cationic, anionic or ampholytic surfactant, preferably a sulfosuccinamate surfactant. The surfactant is the primary collector and the alkoxylated fatty alcohol the secondary collector in the apatite ore flotation process. The degree of branching of the used fatty alcohol is either not disclosed or fatty alcohols are applied which are known to have a degree of branching that is 1 or less. US '466 moreover does not disclose mixtures of two alkoxylated alcohols wherein one is relatively highly branched and ethoxylated with 1 to 4 ethylene oxide groups and the other has a higher amount of EO groups than the first alkoxylated alcohol. Nor does this document disclose the use of such mixtures as secondary collector in the flotation of apatite ores or suggest the benefits thereof.

SE 409291 discloses a method for foam flotation of calcium phosphate-containing minerals, using an amphoteric surface-active compound as the primary collector. The primary collector's flotating ability may further be strengthened by the presence of a secondary collector, which is described as a polar, water-insoluble, hydrophobic substance having affinity to the mineral particles that have been coated by the primary collector. Examples of the polar components are e.g. water-insoluble soaps, such as calcium soaps, water-insoluble surface-active alkylene oxide adducts, organic phosphate compounds, such as tributyl phosphate, and esters of carbonic acids, such as tributyl ester of nitrilotriacetic acid. In the working examples nonylphenol that has been reacted with two moles of ethylene oxide was used as the secondary collector.

The secondary collector disclosed in SE'291 is still considered a good choice in treating ores, as it provides for an excellent mineral recovery at a P₂O₅ grade of higher than 30%. However, due to environmental concerns, an intense search for a replacement of nonylphenol ethoxylates has been ongoing for a long time.

EP 0 270 933 A2 discloses mixtures as collectors for flotation of non-sulfidic ores that contain an alkyl or alkenyl polyethylene glycol ether that is end-capped with a hydrophobic group and an anionic tenside. The end-capped alkyl or alkenyl polyethylene glycol ether in some embodiments is based on a fatty alcohol, preferably a C12 to C18 fatty alcohol. In comparative Examples in EP 0 270 933 also non-end-capped fatty alcohols are used together with anionic tensides. In EP 0 270 933 no disclosure is made of using fatty alcohols having a degree of branching of 1 to 3, and the molecules exemplified in the EP'933 document, though more environmentally friendly than nonylphenol ethoxylates, do not perform as well as these nonylphenol ethoxylates as collectors for flotation of non-sulfidic ores in terms of mineral recovery at the desired high grades.

Thus, there is still a need for secondary collectors having a better environmental profile than nonylphenol ethoxylates that perform equally well.

Shell: "Branching and Carbon Number Type in Detergent Range Alcohols* Branching and Carbon Number Type in Detergent Range Alcohols", of 16 September 2009 discloses the branching of and carbon numbers of Neodol alcohols commercialized by the Shell Group.

Shell: Typical distributions of NEODOL™ ethoxylate adducts" of 5 November 2009 discloses EO distributions of NEODOL ethoxylates commercialized by the Shell Group.

BASF brochure "Lutensol ® TO types" of 28 February 1997 discloses that the Lutensol TO range products are ethoxylated iso C13 alcohols. The degree of ethoxylation of a number of Lutensol^{®} TO products is also disclosed.

Shell brochure: "Neodol 45-7, Primary alcohol ethoxylate" of 1 October 2005 discloses the properties of Neodol 45-7 as commercialized by the Shell Group EP0687726 discloses emulsions of a hydrophilic nonionic surfactant and a hydrophobic nonionic surfactant. The compositions are said to be suitable for the bleaching of fabrics. In one exemplified aqueous formulation with a pH of 4 the surfactants Dobanol 45-7 and Lutensol TO 3 are present together with benzoyl peroxide and sodium coconut alkyl sulfate, and this formulation is employed to bleach a cotton fabric.

US 4,358,368 discloses a process for the froth flotation of calcium phosphate containing minerals using a collector composition that contains an amphoteric surfactant. The surfactant can be combined with a second compound that is hydrophobic and that can be selected from a group of compounds and that is said to be water insoluble. To make the water insoluble secondary compound into a stable emulsion it is suggested that an emulsifier may be added.

Co-pending patent application PCT appl # EP 2015/071003 (published as WO 2016/041916) discloses the use of a secondary collector, suitable for use with a primary collector of the amphoteric or anionic type, for the froth flotation of non-sulfidic ores to recover oxides, carbonates, phosphates and other salt-type minerals, especially calcium phosphate-containing minerals, in which the secondary collector is a branched fatty alcohol-based compound selected from the group of fatty alcohols with 12-16 carbon atoms having a degree of branching of 1-3, and their alkoxylates with a degree of ethoxylation of up to 3.

### Summary of the invention

It has been found in the present invention that a secondary collector which is used in combination with a primary collector of the amphoteric or anionic type for the froth flotation of non-sulfidic ores to recover oxides, carbonates, phosphates and other salt-type minerals, especially calcium phosphate-containing minerals, wherein the secondary collector is a mixture containing at least one compound (i) selected from the group of branched fatty alcohols with 12-16 carbon atoms having a degree of branching of 1-3.5 and their alkoxylates with a degree of ethoxylation (DE) of up to 4, and at least one compound (ii) selected from the group of alkoxylates of nonionic hydrocarbon compounds, such as fatty amines, fatty alcohols, fatty (di)ethanolamides, fatty acids, triglycerides, with a degree of ethoxylation (DE) of higher than 3, leads to similar good efficiency in recovering apatite in the presence of silicate and/or carbonate minerals as when using a secondary collector only containing compound (i), and to the same good environmental profile especially when compared to nonylphenol ethoxylates, but that additionally compound (ii) has as a benefit that it helps to emulsify compound (i) in the collector composition, enabling compound (i) to be used more efficiently, like in a smaller amount.

### Description of the drawings

Figure 1 is the distribution of the degree of ethoxylation in a mixture according to the invention
Figure 2 is a schematic flow chart of a flotation procedure

### Detailed description of the invention

In one aspect, the invention relates to the use of a mixture as a secondary collector for the froth flotation of non-sulfidic ores, in combination with a primary collector selected from the group of amphoteric and anionic surface active compounds, wherein the mixture contains at least one compound (i) selected from the group of branched fatty alcohols with 12-16 carbon atoms having a degree of branching of 1-3.5 and their alkoxylates with a degree of ethoxylation of up to 4, and at least one compound (ii) selected from alkoxylates of nonionic hydrocarbon compounds with a degree of ethoxylation of more than 3, such as alkoxylates of hydrocarbon compounds of the group of fatty alcohols, fatty amines, fatty ethanolamides, fatty diethanolamides, fatty acids, triglycerides with a degree of ethoxylation of more than 3, wherein when both compounds (i) and (ii) are ethoxylated alcohols, the mixture has a bimodal degree of ethoxylation distribution.

It should be noted that the mixture of compounds (i) and (ii) - in the embodiments wherein both compounds are ethoxylated alcohol compounds - has a bimodal DE distribution (bimodal meaning a statistical distribution with two maxima). Or in other words, the mixture is not an inherent mixture of more than one molecule that is obtained when a single ethoxylation reaction is performed with a hydrocarbon compound and wherein always some lower and higher ethoxylated molecules are formed and wherein the DE distribution would be unimodal (i.e. have a single maximum). Instead in the present invention the mixture is a mixture obtained by mixing two separately ethoxylated alcohol compounds (i) and (ii).

If both compounds (i) and (ii) are ethoxylated, preferably the degree of ethoxylation of compound (ii) is higher than that of compound (i).

Additionally, the invention relates to the use of the mixture of the above compounds (i) and (ii) as secondary collectors for the froth flotation of non-sulfidic ores, to recover calcium phosphate-containing minerals, such as apatite, in combination with a primary collector which is an amphoteric or anionic surfactant and to collector compositions containing such primary and secondary collectors. Examples of other valuable minerals that may be recovered using this combination of primary and secondary collectors include scheelite, fluorspar, calcite and dolomite.

In preferred mixtures the ratio of compound (i) to compound (ii) on a weight basis is from 30:70 to 99:1, more preferably from 40:60 to 98:2, even more preferably from 50:50 to 90:10.

By "the degree of branching" (DB) as used herein is meant the total number of methyl groups present on the alkyl or alkenyl chain of the alcohol or alkoxylate thereof, minus one. The mean number of methyl groups in the molecules of a sample can easily be determined by NMR spectroscopy. It should be understood that the degree of branching (DB) in the C12-C16 branched fatty alcohol that delivers the branched alkyl or alkenyl chain for compound (i) is an average degree of branching for the fatty alcohol used. Fatty alcohols are oftentimes available or applied as a mixture of several components and therefore DB does not have to be an integer. Consequently, the degree of branching for compound (i) is an average degree of branching, wherein the average degree of branching is the statistical mean of the degree of branching of the molecules of a sample.

In a preferred embodiment the DB in compound (i) is higher than 1, even more preferably it is higher than 1.5, most preferably higher than 2. In another more preferred embodiment the DB is lower than 3.2, most preferred it is 3 or lower.The molecular formula of the secondary collector compounds (i) and (ii) in a preferred embodiment is

R-A (I),

wherein for compound (i) R is an alkyl or alkenyl group having 12-16, preferably 12-15, carbon atoms and where said alkyl or alkenyl group has a degree of branching of 1-3, and wherein for compound (ii) R is any alkyl, aryl or alkenyl group branched or linear having 8-24 carbon atoms; A is selected from the groups
   O-(PO)ₓ(EO)_{y}(PO)_{z}H, for compounds (i) and (ii)
   (CO)N(CH₂CH₂O(PO)ₓ(EO)_{y}(PO)_{z}H)₂, for compound (ii)
   (CO)NH(CH₂CH₂O(PO)ₓ(EO)_{y}(PO)_{z}H), for compound (ii)
   (CO)O((PO)ₓ(EO)_{y}(PO)_{z}H), for compound (ii)
   N(PO)ₓ(EO)_{y}(PO)_{z}H)₂, for compound (ii), and
   (CO)O((PO)ₓ(EO)_{y}(PO)_{z}OCH₂CH(O(PO)ₓ(EO)_{y}(PO)_{z}O(CO)R)CH₂O((PO)ₓ(EO)_{y}( PO)_{z}O(CO)R), for compound (ii),
wherein for compound (i) PO is a propyleneoxy unit and EO is an ethyleneoxy unit; x is a number 0-2, preferably 0, y is a number 0-4, preferably 0-3, more preferably 0-2.5, even more preferably 0-2.3 and most preferably 0-2, and z is a number 0-2, preferably 0, and wherein for compound (ii) PO is a propyleneoxy unit and EO is an ethyleneoxy unit; x is a number 0-20, preferably 0, y is a number higher than 3 up to 30, preferably 4-20, more preferably 5-15, even more preferably 7-12, z is a number 0-20, preferably 0, and m is an integer of 0 to 5.

The mixture may in addition contain further components such as a liquid. In preferred embodiments such liquid is an aqueous liquid, even more preferably the liquid contains more than 95% of water. In such mixtures compound (ii) acts as an emulsifier for compound (i).

As is evident from formula (I) for compound (i), the alcohols as such, as well as their alkoxylates, may be used in the secondary collector mixtures.

The alkoxylated products according to formula (I) may be produced by procedures well-known in the art by reacting the appropriate starting alcohol, acid, amide, amine or triglyceride with ethylene oxide, or propylene oxide and ethylene oxide, in the presence of a suitable catalyst, e.g. a conventional basic catalyst, such as KOH, or a so-called narrow range catalyst (see e.g. Nonionic Surfactants: Organic Chemistry in Surfactant Science Series volume 72, 1998, pp 1-37 and 87-107, edited by Nico M. van Os; Marcel Dekker, Inc). If both propylene oxide and ethylene oxide are used, the alkoxides may be added as blocks in either order, or may be added randomly. The products obtained from reaction with only ethylene oxide are the most preferred.

Preferred compounds (i) are alcohol alkoxylates with a degree of ethoxylation of up to 3. Preferred compounds (ii) are alcohol alkoxylates with a degree of ethoxylation of higher than 3, even more preferred higher than 4. In an embodiment their degree of ethoxylation is up to 30, preferably up to 20. For both compounds (i) and (ii) it is preferred that they have a degree of propoxylation of less than 2, even more preferably less than 1, most preferably of about 0.

The primary collectors used in the froth flotation according to the present invention may be either amphoteric or anionic surface-active compounds. Below some examples of formulae for the primary collectors are given, but these should only be considered as suitable for the invention, and are not to be regarded as limiting.

In one embodiment the primary collector for the above-mentioned froth flotation procedure has the formula (II)
wherein R₁ is a hydrocarbyl group with 8-22, preferably 12-18, carbon atoms; A is an alkyleneoxy group having 2-4, preferably 2, carbon atoms; p is a number 0 or 1; q is a number from 0 to 5, preferably 0; R₂ is a hydrocarbyl group having 1-4 carbon atoms, preferably 1, or R₂ is the group
wherein R₁, A, p and q have the same meaning as above; Y⁻ is selected from the group consisting of COO⁻ and SO₃⁻, preferably COO⁻; n is a number 1 or 2, preferably 1; M is a cation, which may be monovalent or divalent, and inorganic or organic, and r is a number 1 or 2. The primary collector may also be used in its acid form, where the nitrogen is protonated and no external cation is needed.

The compounds according to formula (II) can easily be produced in high yield from commercially available starting materials using known procedures. US 4,358,368 discloses some ways to produce the compounds where R₁ is a hydrocarbyl group with 8-22 carbon atoms (col 6, line 9 - col 7, line 52), and in US 4,828,687 (col 2, line 2 - col 2, line 31) compounds where R₂ is attached to the compound of formula (II) via the methylene group, are described.

In another embodiment the primary collector has the formula (III) wherein R₂ is a hydrocarbyl group with 8-22, preferably 12-18, carbon atoms, D is -CH₂- or -CH₂CH₂-, k is 0-4, preferably 0-3, and most preferably 0-2, and M is hydrogen or a cation, such as sodium or potassium.

These products are well known and are produced commercially by methods well known in the art. The products where D is -CH₂- are prepared by the reaction between a fatty amine and chloroacetic acid or its salts, and the products where D is -CH₂CH₂- are prepared by the reaction between a fatty amine and acrylic acid or esters thereof, in the latter case the reaction is followed by hydrolysis.

In a further embodiment the primary collector is selected from anionic surface-active compounds such as fatty acids (with a C8 to C24-acyl group), sulfonates, alkyl phosphates, alkyl sulfates and compounds of formula (IV) where R is a hydrocarbyl group having from 7-23, preferably 11-21, carbon atoms, optionally substituted; R₁ is H or CH₃, preferably H; R₂ is H or a C1-C4 alkyl group, preferably H; R₃ is H or CH₃, preferably CH₃; n is a number 1-20; p is a number 1-3, preferably 1; X is H⁺ or a cation which is organic or inorganic, and m represents the valency of the cation and is a number 1-2, preferably 1. The cation is preferably selected from the group consisting of an alkali metal cation, an alkaline earth metal cation, ammonium, and a substituted ammonium group having one or more C₁ to C₃ alkyl and/or hydroxyalkyl groups.

For the production of compounds of formula (IV) see the description in WO 2015/000931 (corresponding to PCT/EP2014/064014).

Also it is possible to have mixtures of the above compounds as a primary collector. In the case of mixing amphoteric and anionic surface-active compounds as the primary collector, it is preferred to have up to 20 weight % of anionic surfactant on the amount of amphoteric surfactant.

In another aspect, the invention relates to a method for froth flotation of non-sulfidic ores, especially phosphate ores, to recover apatite minerals, in which method the collector mixture described above is used.

Such froth flotation method for phosphate ores may typically comprise the steps of:
a) conditioning a pulped ore, wherein the ore comprises a phosphate-containing mineral, and gangue minerals in an aqueous medium, optionally, conditioning the mixture with a flotation aid (in some embodiments a depressant); and optionally, adjusting the pH
b) adding an aqueous composition (in some embodiments an aqueous emulsion) containing the primary and the secondary collector described herein, and, optionally, adjusting the pH
c) optionally, adding a frother; and
d) performing a froth flotation process to recover the phosphate-containing mineral(s).

The weight ratio between the primary collector and the secondary collector in both the collector compositions and the flotation processes is preferably from 15:85, more preferably 20:80, most preferably 25:75 to 99:1, preferably 98:2, most preferably 97:3. All weight ratios herein refer to the ratio of active materials, unless stated otherwise.

The amount of collector composition added to the ore will in general be in the range of from 10 to 1000 g/ton dry ore, preferably in the range of from 20 to 500, more preferably from 100 to 400 g/ton dry ore.

Further flotation aids that may be present in the flotation process are depressants, such as a polysaccharide, alkalized starch or dextrin, extender oils, frothers/froth regulators, such as pine oil, MIBC (methylisobutyl carbinol) and alcohols such as hexanol and alcohol ethoxylates/propoxylates, inorganic dispersants, such as silicate of sodium (water glass) and soda ash, and pH-regulators.

The pH during the flotation process will preferably be in the range of 8-11.

The present invention is further illustrated by the following examples.

### EXAMPLES

### Example 1

### General flotation procedure

A phosphate ore containing 20-25% of apatite, 30-40% of silicates and c. 20% of iron oxides was crushed and ground to a desirable flotation size (K80=110µm).

Three alkoxylates were prepared by reacting the alcohol Exxal 13 (ex Exxon), which has a DB of 3, with ethylene oxide in an amount of 1.5, 5 and 8.5 equivalents, respectively, on the molar amount of the alcohol.

500 g of the ore were placed in a 1.4L Denver flotation cell, 500 ml of process water (25mg/l Ca²⁺, 40mg/l Mg²⁺) were added and the mixing was started. Then 5 minutes conditioning with 1000g/t of a 1%(w/w) aqueous starch solution was performed, the collector (600g/t (or a mixture of primary acylglycide collector and secondary collectors)) was added to the flotation cell as a 1% aqueous solution and conditioning was continued for 2.5 minutes. After the conditioning steps tap water was added so that a total volume of 1.4L was obtained, the pH of the flotation mixture was adjusted to 9.5 with a 10% NaOH aqueous solution and the flotation was started. The experiment was performed at RT (20±1°C).

The rougher flotation, followed by three cleaning steps, was performed. All fractions (tailings, middlings and concentrate) were collected and analysed. Reference is made to Figure 2 for the general procedure that was followed.

The flotation results and the composition of the collector formulation used are displayed in Table 1.

**Table 1. Flotation results presented as P₂O₅ recovery and grade.**

| | Amount of alcohol+XEO, g/t | | | Average degree of ethoxylation | Amount of acylglycide, g/t | 2^{nd} cleaner concentrate | | 3^{rd} cleaner concentrate | |
|---|---|---|---|---|---|---|---|---|---|
| | 1.5EO | 5EO | 8.5EO | | | Recovery, % | Grade, % | Recovery, % | Grade, % |
| Comparison 1 | 0 | 0 | 0 | 0 | 600 | 82.8 | 32.7 | 78.6 | 34.1 |
| Invention | 150 | 0 | 150 | 5 | 300 | 81.6 | 33.2 | 79.5 | 34.2 |
| Comparison 2 | 0 | 300 | 0 | 5 | 300 | 76.6 | 33.4 | 72.4 | 35.0 |

As one can see from Table 1, the flotation results can be improved only if use is made of the mixture of two nonionic surfactants as a secondary collector . In Figure 1 the distribution of the degree of ethoxylation for the formulation according to the invention and the comparison 2 formulation are graphically represented. The results clearly show that the double peak distribution plays a crucial role in the flotation. In a combination with the primary collector the mixture of two ethoxylated alcohols with a degree of ethoxylation equal to 1.5 and 8.5, respectively, provides much better recovery than the single ethoxylated alcohol with a degree of ethoxylation equal to 5.

### Example 2

The emulsion formation and stability were tested by preparing aqueous 5 w% solutions as follows: five (5) g of the surfactant or surfactant mixture were added to 150 ml beaker, diluted with 95 g of water and vigorously mixed. After 5 min the mixing was stopped. Visual observation of the prepared solutions was done after 1, 2, 3, 4, 5, 10 and 60 min.

The results are given in Table 2 below.

**Table 2 Emulsion formation and stability results of mixture of the two alcohol ethoxylates**

| Weight Ratio 1.5EO:8.5EO | Under mixing | 1 min | 2 min | 3 min | 4 min | 5 min | 10 min | 60 min |
|---|---|---|---|---|---|---|---|---|
| 100:0 | 2 p | 2 p | 2 p | 2p | 2 p | 2 p | 2 p | 2 p |
| 90:10 | Em | Em | 2 p | 2 p | 2 p | 2 p | 2 p | 2 p |
| 80:20 | Em | Em | Em | Em | 2 p | 2 p | 2 p | 2 p |
| 50:50 | Em | Em | Em | Em | Em | Em | Em | 2 p |

| | | | | | | | | |
|---|---|---|---|---|---|---|---|---|
| Em means emulsion, 2p means 2 phases | | | | | | | | |

From Table 2 it is clear that adding a compound having a degree of ethoxylation of higher than 3 to an alcohol ethoxylate that only has a degree of ethoxylation of 1.5 helps considerably to form an emulsion. Adding more of the higher ethoxylated product such as up to 50 wt% makes the emulsion much more stable.

## Claims

1. Use of a mixture as secondary collector for the froth flotation of non-sulfidic ores, in combination with a primary collector selected from the group of amphoteric and anionic surface active compounds, wherein the mixture contains at least one compound (i) selected from the group of alkoxylates of branched fatty alcohols with 12-16 carbon atoms having a degree of branching of 1-3.5, with a degree of ethoxylation of up to 4 and at least one compound (ii) selected from the group of alkoxylates of nonionic hydrocarbon compounds with a degree of ethoxylation of higher than 3, wherein if both compounds (i) and (ii) are ethoxylated alcohols, the mixture has a bimodal degree of ethoxylation distribution.

2. Use of claim 1 wherein the compound (ii) is selected from the group of alkoxylates of nonionic hydrocarbon compounds from the group of fatty alcohols, fatty amines, fatty ethanolamides, fatty diethanolamides, fatty acids, and triglycerides with a degree of ethoxylation of more than 3.

3. Use according to claim 1 or 2 where the molecular formula of compound (i) and (ii) is of the formula (I)
R-A (I)
wherein for compound (i) R is an alkyl or alkenyl group having 12-16, preferably 12-15, carbon atoms, and where said alkyl or alkenyl group has a degree of branching of 1-3 and wherein for compound (ii) R is any alkyl, aryl or alkenyl group branched or linear having 8-24 carbon atoms; A is selected from the groups
O-(PO)ₓ(EO)_{y}(PO)_{z}H, for compounds (i) and (ii)
(CO)N(CH₂CH₂O(PO)ₓ(EO)_{y}(PO)_{z}H)₂, for compound (ii)
(CO)NH(CH₂CH₂O(PO)ₓ(EO)_{y}(PO)_{z}H), for compound (ii)
(CO)O((PO)ₓ(EO)_{y}(PO)_{z}H), for compound (ii)
N(PO)ₓ(EO)_{y}(PO)_{z}H)₂, for compound (ii)
(CO)O((PO)ₓ(EO)_{y}(PO)_{z}OCH₂CH(O(PO)ₓ(EO)_{y}(PO)_{z}O(CO)R)CH₂O and
((PO)ₓ(EO)_{y}(PO)_{z}O(CO)R), for compound (ii),
wherein PO is a propyleneoxy unit and EO is an ethyleneoxy unit and for compound (i); x is a number 0-2, preferably 0, y is a number 0-4, preferably 0-3, more preferably 0-2.5, even more preferably 0-2.3 and most preferably 0-2, and z is a number 0-2, preferably 0, and for compound (ii) x is a number 0-20, preferably 0, y is a number higher than 3 up to 30, preferably 4-20, more preferably 5-15, even more preferably 7-12, and z is a number 0-20, preferably 0.

4. Use of any one of claims 1 to 3 wherein the mixture additionally contains a liquid wherein compound (ii) is an emulsifier for compound (i) in the liquid

5. Use according to any one of claims 1to 4 wherein said primary collector is an amphoteric surface-active compound selected from the group consisting of compounds having the formula (II)
wherein R₁ is a hydrocarbyl group with 8-22, preferably 12-18, carbon atoms; A is an alkyleneoxy group having 2-4 carbon atoms; p is a number 0 or 1; q is a number from 0 to 5, preferably 0, R₂ is a hydrocarbyl group having 1-4 carbon atoms, preferably 1, or R₂ is the group ,
wherein R₁, A, p and q have the same meaning as above, Y⁻ is selected from the group consisting of COO⁻ and SO₃⁻, preferably COO⁻; n is a number 1 or 2, preferably 1; M is a cation which may be monovalent or divalent and inorganic or organic, and r is a number 1 or 2; or where the compound (II) is in its acidic protonated form without an external cation (M^{r+}) 1/r; and compounds having the formula (III)
wherein R₂ is a hydrocarbyl group with 8-22, preferably 12-18, carbon atoms, D is -CH₂- or -CH₂CH₂-, k is 0-4, preferably 0-3, and most preferably 0-2, and M is hydrogen or a cation, such as sodium or potassium, and
anionic surface-active compound selected from the group consisting of fatty acids, sulfonates, alkyl phosphates, alkyl sulfates and compounds of formula (IV)
wherein R is a hydrocarbyl group having from 7-23, preferably 11-21, carbon atoms, optionally substituted; R₁ is H or CH₃, preferably H; R₂ is H or a C1-C4 alkyl group, preferably H; R₃ is H or CH₃, preferably CH₃; n is a number 1-20; p is a number 1-3, preferably 1; X is H⁺ or a cation which is organic or inorganic, and m represents the valency of the cation and is a number 1-2, preferably 1, and mixtures thereof.

6. Use according to any one of the preceding claims 1 to 5 wherein the weight ratio between the primary collector and the secondary collector is between 15:85 and 99:1.

7. Use according to any one of the preceding claims 1 to 6 wherein the non-sulfidic ore is a calcium phosphate-containing ore.

8. A process for the froth flotation of non-sulfidic ores using a collector composition comprising a primary collector selected from the group of amphoteric and anionic surface-active compounds, and a secondary collector that contains a mixture containing at least one compound (i) selected from the group of alkoxylates of branched fatty alcohols with 12-16 carbon atoms having a degree of branching of 1-3.5, with a degree of ethoxylation of up to 4 and at least one compound (ii) selected from the group of alkoxylates of nonionic hydrocarbon compounds, with a degree of ethoxylation of higher than 3, wherein if both compounds (i) and (ii) are ethoxylated alcohols, the mixture has a bimodal degree of ethoxylation distribution.

9. A process for the froth flotation of non-sulfidic ores according to claim 8 wherein the compound (ii) is selected from the group of alkoxylates of nonionic hydrocarbon compounds from the group of fatty alcohols, fatty amines, fatty ethanolamides, fatty diethanolamides, fatty acids, and triglycerides with a degree of ethoxylation of more than 3.

10. The process according to claim 8 or 9 where the molecular formula of compound (i) and (ii) is of the formula (I)
R-A (I)
wherein for compound (i) R is an alkyl or alkenyl group having 12-16, preferably 12-15, carbon atoms, and where said alkyl or alkenyl group has a degree of branching of 1-3 and wherein for compound (ii) R is any alkyl, aryl or alkenyl group branched or linear having 8-24 carbon atoms; A is selected from the groups
O-(PO)ₓ(EO)_{y}(PO)_{z}H, for compounds (i) and (ii)
(CO)N(CH₂CH₂O(PO)ₓ(EO)_{y}(PO)_{z}H)₂, for compound (ii)
(CO)NH(CH₂CH₂O(PO)ₓ(EO)_{y}(PO)_{z}H), for compound (ii)
(CO)O((PO)ₓ(EO)_{y}(PO)_{z}H), for compound (ii)
N(PO)ₓ(EO)_{y}(PO)_{z}H)₂, for compound (ii)
(CO)O((PO)ₓ(EO)_{y}(PO)_{z}OCH₂CH(O(PO)ₓ(EO)_{y}(PO)_{z}O(CO)R)CH₂O, and
((PO)ₓ(EO)_{y}(PO)_{z}O(CO)R), for compound (ii),
wherein PO is a propyleneoxy unit and EO is an ethyleneoxy unit and for compound (i); x is a number 0-2, preferably 0, y is a number 0-4, preferably 0-3, more preferably 0-2.5, even more preferably 0-2.3 and most preferably 0-2, and z is a number 0-2, preferably 0, and for compound (ii) x is a number 0-20, preferably 0, y is a number higher than 3 up to 30, preferably 4-20, more preferably 5-15, even more preferably 7-12, and z is a number 0-20, preferably 0.

11. A process according to any one of claims 8 to 10 which comprises the steps
i) conditioning a pulped non-sulfidic ore, wherein the ore comprises a phosphate-containing mineral, and gangue minerals, with the collector composition , and optionally other flotation aids and
ii) performing a froth flotation process to recover the phosphate-containing mineral(s).

12. The process according to any one of claims 8 to 11 wherein said primary collector is an amphoteric surface-active compounds selected from the group consisting of compounds having the formula (II)
wherein R₁ is a hydrocarbyl group with 8-22, preferably 12-18, carbon atoms; A is an alkyleneoxy group having 2-4 carbon atoms; p is a number 0 or 1; q is a number from 0 to 5, preferably 0; R₂ is a hydrocarbyl group having 1-4 carbon atoms, preferably 1, or R₂ is the group ,
wherein R₁, A, p and q have the same meaning as above, Y⁻ is selected from the group consisting of COO⁻ and SO₃⁻, preferably COO⁻; n is a number 1 or 2, preferably 1; M is a cation which may be monovalent or divalent and inorganic or organic, and r is a number 1 or 2; or where the compound (II) is in its acidic protonated form without an external cation (M^{r+}) 1/r; and
compounds of formula (III)
wherein R₂ is a hydrocarbyl group with 8-22, preferably 12-18, carbon atoms, D is -CH₂- or -CH₂CH₂-, k is 0-4, preferably 0-3, and most preferably 0-2, and M is hydrogen or a cation, such as sodium or potassium; or.
an anionic surface-active compound selected from the group consisting of fatty acids, sulfonates, alkyl phosphates, alkyl sulfates and compounds of formula (IV)
wherein R is a hydrocarbyl group having from 7-23, preferably 11-21, carbon atoms, optionally substituted; R₁ is H or CH₃, preferably H; R₂ is H or a C1-C4 alkyl group, preferably H; R₃ is H or CH₃, preferably CH₃; n is a number 1-20; p is a number 1-3, preferably 1; X is H⁺ or a cation which is organic or inorganic, and m represents the valency of the cation and is a number 1-2, preferably 1; and mixtures thereof.

13. A process according to any one of claims 8 to 12 wherein the weight ratio between the primary collector and the secondary collector is from 15:85 to 99:1.

## Patentansprüche

1. Verwendung einer Mischung eines sekundären Sammlers für die Schaumflotation nichtsulfidischer Erze in Kombination mit einem primären Sammler ausgewählt aus der Gruppe von amphoteren und anionischen oberflächenaktiven Verbindungen, wobei die Mischung mindestens eine Verbindung (i) ausgewählt aus der Gruppe von Alkoxylaten verzweigter Fettalkohole mit 12-16 Kohlenstoffatomen, die einen Verzweigungsgrad von 1-3,5 aufweisen, mit einem Ethoxylierungsgrad von bis zu 4 und mindestens eine Verbindung (ii) enthält ausgewählt aus der Gruppe von Alkoxylaten nichtionischer Kohlenwasserstoffverbindungen mit einem Ethoxylierungsgrad höher als 3, wobei, wenn beide Verbindungen (i) und (ii) ethoxylierte Alkohole sind, die Mischung einen bimodalen Ethoxylierungsverteilungsgrad aufweist.

2. Verwendung nach Anspruch 1, wobei die Verbindung (ii) aus der Gruppe ausgewählt ist von Alkoxylaten nichtionischer Kohlenwasserstoffverbindungen aus der Gruppe von Fettalkoholen, Fettaminen, Fettethanolamiden, Fettdiethanolamiden, Fettsäuren und Triglyceriden mit einem Ethoxylierungsgrad von mehr als 3.

3. Verwendung nach Anspruch 1 oder 2, wobei die Molekülformel der Verbindungen (i) und (ii) die Formel (I) aufweist
R-A (I),
wobei, für die Verbindung (i), R eine Alkyl- oder Alkenylgruppe ist, die 12-16, bevorzugt 12-15, Kohlenstoffatome aufweist und wobei die Alkyl- oder Alkenylgruppe einen Verzweigungsgrad von 1-3 aufweist und wobei, für die Verbindung (ii), R irgendeine verzweigte oder lineare Alkyl-, Aryl- oder Alkenylgruppe ist, die 8-24 Kohlenstoffatome aufweist;
A aus den Gruppen ausgewählt ist
O-(PO)ₓ(EO)_{y}(PO)_{z}H für die Verbindungen (i) und (ii) (CO)N(CH₂CH₂O(PO)ₓ(EO)_{y}(PO)_{z}H)₂ für die Verbindung (ii) (CO)NH(CH₂CH₂O(PO)ₓ(EO)_{y}(PO)₂H) für die Verbindung (ii) (CO)O((PO)ₓ(EO)_{y}(PO)_{z}H) für die Verbindung (ii) N(PO)ₓ(EO)_{y}(PO)_{z}H)₂ für die Verbindung (ii)
(CO)O((PO)ₓ(EO)_{y}(PO)_{z}OCH₂CH(O(PO)ₓ(EO)_{y}(PO)_{z}O(CO)R)CH₂O und
((PO)ₓ(EO)_{y}(PO)_{z}O(CO)R) für die Verbindung (ii),
wobei PO eine Propylenoxyeinheit ist und EO eine Ethylenoxyeinheit ist und für die Verbindung (i): x eine Zahl von 0-2, bevorzugt 0, ist, y eine Zahl von 0-4, bevorzugt 0-3, noch bevorzugter 0-2,5, selbst noch bevorzugter 0-2,3 und am bevorzugtesten 0-2 ist und z eine Zahl von 0-2, bevorzugt 0 ist und für die Verbindung (ii) x eine Zahl von 0-20, bevorzugt 0 ist, y eine Zahl höher als 3 bis zu 30, bevorzugt 4-20, noch bevorzugter 5-15, selbst noch bevorzugter 7-12 ist und z eine Zahl von 0-20, bevorzugt 0 ist.

4. Verwendung nach einem der Ansprüche 1 bis 3, wobei die Mischung zusätzlich eine Flüssigkeit enthält, wobei die Verbindung (ii) ein Emulator für die Verbindung (i) in der Flüssigkeit ist.

5. Verwendung nach einem der Ansprüche 1 bis 4, wobei der primäre Sammler eine amphotere oberflächenaktive Verbindung ist ausgewählt aus der Gruppe bestehend aus Verbindungen, die die Formel (II) aufweisen
wobei R₁ eine Hydrocarbylgruppe mit 8-22, bevorzugt 12-18, Kohlenstoffatomen ist; A eine Alkylenoxygruppe ist, die 2-4 Kohlenstoffatome aufweist; p eine Zahl von 0 oder 1 ist; q eine Zahl von 0 bis 5, bevorzugt 0, ist; R₂ eine Hydrocarbylgruppe ist, die 1-4 Kohlenstoffatome, bevorzugt 1, aufweist oder R₂ die Gruppe ist
wobei R₁, A, p und q dieselbe Bedeutung wie oben besitzen, Y⁻ aus der Gruppe ausgewählt ist bestehend aus COO⁻ und SO₃⁻, bevorzugt COO⁻; n eine Zahl von 1 oder 2, bevorzugt 1, ist; M ein Kation ist, das einwertig oder zweiwertig und anorganisch oder organisch sein kann, und r eine Zahl von 1 oder 2 ist; oder wobei die Verbindung (II) in ihrer sauren protonierten Form ohne ein externes Kation (M^{r+})1/r vorliegt; und Verbindungen, die die Formel (III) aufweisen
wobei R₂ eine Hydrocarbylgruppe mit 8-22, bevorzugt 12-18, Kohlenstoffatomen ist; D -CH₂- oder -CH₂CH₂- ist, k 0-4, bevorzugt 0-3 und am bevorzugtesten 0-2 beträgt und M Wasserstoff oder ein Kation, wie beispielsweise Natrium oder Kalium, ist und
einer anionischen oberflächenaktiven Verbindung ausgewählt aus der Gruppe bestehend aus Fettsäuren, Sulfonaten, Alkylphosphaten, Alkylsulfaten und Verbindungen der Formel (IV)
wobei R eine Hydrocarbylgruppe ist, die 7-23, bevorzugt 11-21, Kohlenstoffatome aufweist, die wahlweise substituiert sind; R₁ H oder CH₃, bevorzugt H, ist; R₂ H oder eine C1-C4-Alkylgruppe, bevorzugt H, ist; R₃ H oder CH₃, bevorzugt CH₃ ist; n eine Zahl von 1-20 ist; p eine Zahl von 1-3, bevorzugt 1 ist; X H⁺ oder ein Kation ist, das organisch oder anorganisch ist, und m die Wertigkeit des Kations darstellt und eine Zahl von 1-2, bevorzugt 1, ist, und Mischungen davon.

6. Verwendung nach einem der vorhergehenden Ansprüche 1 bis 5, wobei das Gewichtsverhältnis zwischen dem primären Sammler und dem sekundären Sammler zwischen 15:85 und 99:1 liegt.

7. Verwendung nach einem der vorhergehenden Ansprüche 1 bis 6, wobei das nichtsulfidische Erz ein Calciumphosphat enthaltendes Erz ist.

8. Verfahren für die Schaumflotation nichtsulfidischer Erze unter Verwendung einer Sammlerzusammensetzung umfassend einen primären Sammler ausgewählt aus der Gruppe von amphoteren und anionischen oberflächenaktiven Verbindungen und einen sekundären Sammler, der eine Mischung enthält, die mindestens eine Verbindung (i) ausgewählt aus der Gruppe von Alkoxylaten verzweigter Fettalkohole mit 12-16 Kohlenstoffatomen, die einen Verzweigungsgrad von 1-3,5 aufweisen, mit einem Ethoxylierungsgrad von bis zu 4 und mindestens eine Verbindung (ii) enthält ausgewählt aus der Gruppe von Alkoxylaten nichtionischer Kohlenwasserstoffverbindungen mit einem Ethoxylierungsgrad höher als 3, wobei, wenn beide Verbindungen (i) und (ii) ethoxylierte Alkohole sind, die Mischung einen bimodalen Ethoxylierungsverteilungsgrad aufweist.

9. Verfahren für die Schaumflotation nichtsulfidischer Erze nach Anspruch 8, wobei die Verbindung (ii) aus der Gruppe ausgewählt ist von Alkoxylaten nichtionischer Kohlenwasserstoffverbindungen der Gruppe von Fettalkoholen, Fettaminen, Fettethanolamiden, Fettdiethanolamiden, Fettsäuren und Triglyceriden mit einem Ethoxylierungsgrad von mehr als 3.

10. Verfahren nach Anspruch 8 oder 9, wobei die Molekülformel der Verbindungen (i) und (ii) die Formel (I) aufweist
R-A (I)
ist,
wobei, für die Verbindung (i), R eine Alkyl- oder Alkenylgruppe ist, die 12-16, bevorzugt 12-15, Kohlenstoffatome aufweist und wobei die Alkyl- oder Alkenylgruppe einen Verzweigungsgrad von 1-3 aufweist und wobei für die Verbindung (ii) R irgendeine verzweigte oder lineare Alkyl-, Aryl- oder Alkenylgruppe ist, die 8-24 Kohlenstoffatome aufweist;
A aus den Gruppen ausgewählt ist
O-(PO)ₓ(EO)_{y}(PO)_{z}H für die Verbindungen (i) und (ii) (CO)N(CH₂CH₂O(PO)ₓ(EO)_{y}(PO)_{z}H)₂ für die Verbindung (ii) (CO)NH(CH₂CH₂O(PO)ₓ(EO)_{y}(PO)_{z}H) für die Verbindung (ii) (CO)O((PO)ₓ(EO)_{y}(PO)_{z}H) für die Verbindung (ii) N(PO)ₓ(EO)_{y}(PO)_{z}H)₂ für die Verbindung (ii)
(CO)O((PO)ₓ(EO)_{y}(PO)_{z}OCH₂CH(O(PO)ₓ(EO)_{y}(PO)_{z}O(CO)R)CH₂O
und
((PO)ₓ(EO)_{y}(PO)_{z}O(CO)R) für die Verbindung (ii),
wobei PO eine Propylenoxyeinheit ist und EO eine Ethylenoxyeinheit ist und für die Verbindung (i): x eine Zahl von 0-2, bevorzugt 0, ist, y eine Zahl von 0-4, bevorzugt 0-3, noch bevorzugter 0-2,5, selbst noch bevorzugter 0-2,3 und am bevorzugtesten 0-2 ist und z eine Zahl von 0-2, bevorzugt 0 ist und für die Verbindung (ii) x eine Zahl von 0-20, bevorzugt 0 ist, y eine Zahl höher als 3 bis zu 30, bevorzugt 4-20, noch bevorzugter 5-15, selbst noch bevorzugter 7-12 ist und z eine Zahl von 0-20, bevorzugt 0 ist.

11. Verfahren nach einem der Ansprüche 8 bis 10, das die Schritte umfasst
i) Konditionieren eines zerkleinerten nichtsulfidischen Erzes, wobei das Erz ein phosphathaltiges Mineral und Gangmineralien umfasst, mit der Sammlerzusammensetzung und wahlweise anderen Flotationshilfsmitteln und
ii) Ausführen eines Schaumflotationsverfahrens, um das/die phosphathaltige(n) Mineral(ien) zu gewinnen.

12. Verfahren nach einem der Ansprüche 8 bis 11, wobei der primäre Sammler eine amphotere oberflächenaktive Verbindung ist ausgewählt aus der Gruppe bestehend aus Verbindungen, die die Formel (II) aufweisen
wobei R₁ eine Hydrocarbylgruppe mit 8-22, bevorzugt 12-18, Kohlenstoffatomen ist; A eine Alkylenoxygruppe ist, die 2-4 Kohlenstoffatome aufweist; p eine Zahl von 0 oder 1 ist; q eine Zahl von 0 bis 5, bevorzugt 0, ist; R₂ eine Hydrocarbylgruppe ist, die 1-4 Kohlenstoffatome, bevorzugt 1, aufweist oder R₂ die Gruppe ist
wobei R₁, A, p und q dieselbe Bedeutung wie oben besitzen, Y⁻ aus der Gruppe ausgewählt ist bestehend aus COO⁻ und SO₃⁻, bevorzugt COO⁻; n eine Zahl von 1 oder 2, bevorzugt 1, ist; M ein Kation ist, das einwertig oder zweiwertig und anorganisch oder organisch sein kann, und r eine Zahl von 1 oder 2 ist; oder wobei die Verbindung (II) in ihrer sauren protonierten Form ohne ein externes Kation (M^{r+})1/r vorliegt; und
Verbindungen, die die Formel (III) aufweisen
wobei R₂ eine Hydrocarbylgruppe mit 8-22, bevorzugt 12-18, Kohlenstoffatomen ist; D -CH₂- oder -CH₂CH₂- ist, k 0-4, bevorzugt 0-3 und am bevorzugtesten 0-2 beträgt und M Wasserstoff oder ein Kation, wie beispielsweise Natrium oder Kalium, ist; oder
einer anionischen oberflächenaktiven Verbindung ausgewählt aus der Gruppe bestehend aus Fettsäuren, Sulfonaten, Alkylphosphaten, Alkylsulfaten und Verbindungen der Formel (IV)
wobei R eine Hydrocarbylgruppe ist, die 7-23, bevorzugt 11-21, Kohlenstoffatome aufweist, die wahlweise substituiert sind; R₁ H oder CH₃, bevorzugt H, ist; R₂ H oder eine C1-C-Alkylgruppe, bevorzugt H, ist; R₃ H oder CH₃, bevorzugt CH₃ ist; n eine Zahl von 1-20 ist; p eine Zahl von 1-3, bevorzugt 1, ist; X H⁺ oder ein Kation ist, das organisch oder anorganisch ist, und m die Wertigkeit des Kations darstellt und eine Zahl von 1-2, bevorzugt 1 ist, und Mischungen davon.

13. Verfahren nach einem der Ansprüche 8 bis 12, wobei das Gewichtsverhältnis zwischen dem primären Sammler und dem sekundären Sammler 15:85 bis 99:1 beträgt.

## Revendications

1. Utilisation d'un mélange en tant que collecteur secondaire pour la flottation par moussage de minerais non sulfurés, en combinaison avec un collecteur primaire sélectionné dans le groupe des composés tensioactifs amphotères et anioniques, dans laquelle le mélange contient au moins un composé (i) sélectionné dans le groupe des alcoxylates d'alcools gras ramifiés comprenant de 12 à 16 atomes de carbone ayant un degré de ramification de 1 à 3,5, avec un degré d'éthoxylation allant jusqu'à 4 et au moins un composé (ii) sélectionné dans le groupe des alcoxylates de composés hydrocarbonés non ioniques avec un degré d'éthoxylation supérieur à 3, dans laquelle si les deux composés (i) et (ii) sont des alcools éthoxylés, le mélange présente un degré bimodal de distribution d'éthoxylation.

2. Utilisation selon la revendication 1 dans laquelle le composé (ii) est sélectionné dans le groupe des alcoxylates de composés hydrocarbonés non ioniques du groupe des alcools gras, des aminés grasses, des éthanolamides gras, des diéthanolamides gras, des acides gras et des triglycérides avec un degré d'éthoxylation supérieur à 3.

3. Utilisation selon la revendication 1 ou 2 où la formule moléculaire des composés (i) et (ii) répond à la formule (I)
R-A (I)
dans laquelle pour le composé (i) R est un groupe alkyle ou alcényle comprenant de 12 à 16, de préférence de 12 à 15, atomes de carbone, et où ledit groupe alkyle ou alcényle a un degré de ramification de 1 à 3, et dans laquelle pour le composé (ii) R est n'importe quel groupe alkyle, aryle ou alcényle ramifié ou linéaire comprenant de 8 à 24 atomes de carbone ; A est sélectionné parmi les groupes O-(PO)ₓ(EO)_{y}(PO)_{z}H, pour les composés (i) et (ii)
(CO)N(CH₂CH₂O(PO)ₓ(EO)_{y}(PO)_{z}H)₂, pour le composé (ii)
(CO)NH(CH₂CH₂O(PO)ₓ(EO)_{y}(PO)_{z}H), pour le composé (ii)
(CO)O((PO)ₓ(EO)_{y}(PO)_{z}H), pour le composé (ii)
N(PO)ₓ(EO)_{y}(PO)_{z}H)₂, pour le composé (ii)
(CO)O((PO)ₓ(EO)_{y}(PO)_{z}OCH₂CH(O(PO)ₓ(EO)_{y}(PO)_{z}O(CO)R)CH₂O et
((PO)ₓ(EO)_{y}(PO)_{z}O(CO)R), pour le composé (ii),
dans laquelle PO est un motif propylèneoxy et EO est un motif éthylèneoxy, et pour le composé (i) ; x est un nombre de 0 à 2, de préférence égal à 0, y est un nombre de 0 à 4, de préférence de 0 à 3, plus préférablement de 0 à 2,5, encore plus préférablement de 0 à 2,3 et de manière préférée entre toutes de 0 à 2, et z est un nombre de 0 à 2, de préférence égal à 0, et pour le composé (ii) x est un nombre de 0 à 20, de préférence égal à 0, y est un nombre supérieur à 3 allant jusqu'à 30, de préférence de 4 à 20, plus préférablement de 5 à 15, encore plus préférablement de 7 à 12, et z est un nombre de 0 à 20, de préférence égal à 0.

4. Utilisation selon l'une quelconque des revendications 1 à 3 dans laquelle le mélange contient en outre un liquide dans laquelle le composé (ii) est un émulsifiant pour le composé (i) dans le liquide.

5. Utilisation selon l'une quelconque des revendications 1 à 4 dans laquelle ledit collecteur primaire est un composé tensioactif amphotère sélectionné dans le groupe constitué par les composés répondant à la formule (II)
dans laquelle R₁ est un groupe hydrocarbyle comprenant de 8 à 22, de préférence de 12 à 18, atomes de carbone ; A est un groupe alkylèneoxy comprenant de 2 à 4 atomes de carbone ; p est un nombre égal à 0 ou 1 ; q est un nombre de 0 à 5, de préférence égal à 0, R₂ est un groupe hydrocarbyle comprenant de 1 à 4 atomes de carbone, de préférence 1, ou R₂ est le groupe
dans lequel R₁, A, p et q ont la même signification que ci-dessus, Y⁻ est sélectionné dans le groupe constitué par COO⁻ et SO₃⁻, de préférence COO⁻ ; n est un nombre égal à 1 ou 2, de préférence égal à 1 ; M est un cation qui peut être monovalent ou divalent et inorganique ou organique, et r est un nombre égal à 1 ou 2 ; ou lorsque le composé (II) est sous sa forme protonée acide sans cation externe (M^{r+}) 1/r ; et les composés répondant à la formule (III)
dans laquelle R₂ est un groupe hydrocarbyle comprenant de 8 à 22, de préférence de 12 à 18, atomes de carbone, D est -CH₂- ou -CH₂CH₂-, k vaut de 0 à 4, de préférence de 0 à 3, et de manière préférée entre toutes de 0 à 2, et M est un atome d'hydrogène ou un cation, tel que le sodium ou le potassium, et
un composé tensioactif anionique sélectionné dans le groupe constitué par les acides gras, les sulfonates, les alkylphosphates, les alkylsulfates et les composés de formule (IV)
dans laquelle R est un groupe hydrocarbyle comprenant de 7 à 23, de préférence de 11 à 21, atomes de carbone, éventuellement substitué ; R₁ est H ou CH₃, de préférence H ; R₂ est H ou un groupe alkyle en C1 à C4, de préférence H ; R₃ est H ou CH₃, de préférence CH₃ ; n est un nombre de 1 à 20 ; p est un nombre de 1 à 3, de préférence égal à 1 ; X est H⁺ ou un cation qui est organique ou inorganique, et m représente la valence du cation et est un nombre de 1 à 2, de préférence égal à 1, et des mélanges de ceux-ci.

6. Utilisation selon l'une quelconque des revendications 1 à 5 précédentes dans laquelle le rapport pondéral entre le collecteur primaire et le collecteur secondaire est compris entre 15:85 et 99:1.

7. Utilisation selon l'une quelconque des revendications 1 à 6 précédentes dans laquelle le minerai non sulfuré est un minerai contenant du phosphate de calcium.

8. Procédé pour la flottation par moussage de minerais non sulfurés utilisant une composition collectrice comprenant un collecteur primaire sélectionné dans le groupe des composés tensioactifs amphotères et anioniques, et un collecteur secondaire qui contient un mélange contenant au moins un composé (i) sélectionné dans le groupe des alcoxylates d'alcools gras ramifiés comprenant de 12 à 16 atomes de carbone ayant un degré de ramification de 1 à 3,5, avec un degré d'éthoxylation allant jusqu'à 4, et au moins un composé (ii) sélectionné dans le groupe des alcoxylates de composés hydrocarbonés non ioniques, avec un degré d'éthoxylation supérieur à 3, dans lequel si les deux composés (i) et (ii) sont des alcools éthoxylés, le mélange présente un degré bimodal de distribution d'éthoxylation.

9. Procédé pour la flottation par moussage de minerais non sulfurés selon la revendication 8 dans lequel le composé (ii) est sélectionné dans le groupe des alcoxylates de composés hydrocarbonés non ioniques du groupe des alcools gras, des aminés grasses, des éthanolamides gras, des diéthanolamides gras, des acides gras et des triglycérides avec un degré d'éthoxylation supérieur à 3.

10. Procédé selon la revendication 8 ou 9 où la formule moléculaire des composés (i) et (ii) répond à la formule (I)
R-A (I)
dans laquelle pour le composé (i) R est un groupe alkyle ou alcényle comprenant de 12 à 16, de préférence de 12 à 15, atomes de carbone, et où ledit groupe alkyle ou alcényle a un degré de ramification de 1 à 3, et dans laquelle pour le composé (ii) R est n'importe quel groupe alkyle, aryle ou alcényle ramifié ou linéaire comprenant de 8 à 24 atomes de carbone ; A est sélectionné parmi les groupes
O-(PO)ₓ(EO)_{y}(PO)_{z}H, pour les composés (i) et (ii)
(CO)N(CH₂CH₂O(PO)ₓ(EO)_{y}(PO)_{z}H)₂, pour le composé (ii)
(CO)NH(CH₂CH₂O(PO)ₓ(EO)_{y}(PO)_{z}H), pour le composé (ii)
(CO)O((PO)ₓ(EO)_{y}(PO)_{z}H), pour le composé (ii)
N(PO)ₓ(EO)_{y}(PO)_{z}H)₂, pour le composé (ii)
(CO)O((PO)ₓ(EO)_{y}(PO)_{z}OCH₂CH(O(PO)ₓ(EO)_{y}(PO)_{z}O(CO)R)CH₂O et
((PO)ₓ(EO)_{y}(PO)_{z}O(CO)R), pour le composé (ii),
dans laquelle PO est un motif propylèneoxy et EO est un motif éthylèneoxy, et pour le composé (i) ; x est un nombre de 0 à 2, de préférence égal à 0, y est un nombre de 0 à 4, de préférence de 0 à 3, plus préférablement de 0 à 2,5, encore plus préférablement de 0 à 2,3 et de manière préférée entre toutes de 0 à 2, et z est un nombre de 0 à 2, de préférence égal à 0, et pour le composé (ii) x est un nombre de 0 à 20, de préférence égal à 0, y est un nombre supérieur à 3 allant jusqu'à 30, de préférence de 4 à 20, plus préférablement de 5 à 15, encore plus préférablement de 7 à 12, et z est un nombre de 0 à 20, de préférence égal à 0.

11. Procédé selon l'une quelconque des revendications 8 à 10 qui comprend les étapes
i) conditionnement d'un minerai non sulfuré sous forme de pâte, dans lequel le minerai comprend un minéral contenant du phosphate, et des minéraux de la gangue, avec la composition collectrice, et éventuellement d'autres adjuvants de flottation et
ii) mise en œuvre d'un procédé de flottation par moussage pour récupérer le ou les minéraux contenant du phosphate.

12. Procédé selon l'une quelconque des revendications 8 à 11 dans lequel ledit collecteur primaire est un composé tensioactif amphotère sélectionné dans le groupe constitué par les composés répondant à la formule (II)
dans laquelle R₁ est un groupe hydrocarbyle comprenant de 8 à 22, de préférence de 12 à 18, atomes de carbone ; A est un groupe alkylèneoxy comprenant de 2 à 4 atomes de carbone ; p est un nombre égal à 0 ou 1 ; q est un nombre de 0 à 5, de préférence égal à 0 ; R₂ est un groupe hydrocarbyle comprenant de 1 à 4 atomes de carbone, de préférence 1, ou R₂ est le groupe
dans lequel R₁, A, p et q ont la même signification que ci-dessus, Y⁻ est sélectionné dans le groupe constitué par COO⁻ et SO₃⁻, de préférence COO⁻ ; n est un nombre égal à 1 ou 2, de préférence égal à 1 ; M est un cation qui peut être monovalent ou divalent et inorganique ou organique, et r est un nombre égal à 1 ou 2 ; ou lorsque le composé (II) est sous sa forme protonée acide sans cation externe (M^{r+}) 1/r ; et les composés répondant à la formule (III)
dans laquelle R₂ est un groupe hydrocarbyle comprenant de 8 à 22, de préférence de 12 à 18, atomes de carbone, D est -CH₂- ou -CH₂CH₂-, k vaut de 0 à 4, de préférence de 0 à 3, et de manière préférée entre toutes de 0 à 2, et M est un atome d'hydrogène ou un cation, tel que le sodium ou le potassium ; ou
un composé tensioactif anionique sélectionné dans le groupe constitué par les acides gras, les sulfonates, les alkylphosphates, les alkylsulfates et les composés de formule (IV)
dans laquelle R est un groupe hydrocarbyle comprenant de 7 à 23, de préférence de 11 à 21, atomes de carbone, éventuellement substitué ; R₁ est H ou CH₃, de préférence H ; R₂ est H ou un groupe alkyle en C1 à C4, de préférence H ; R₃ est H ou CH₃, de préférence CH₃ ; n est un nombre de 1 à 20 ; p est un nombre de 1 à 3, de préférence égal à 1 ; X est H⁺ ou un cation qui est organique ou inorganique, et m représente la valence du cation et est un nombre de 1 à 2, de préférence égal à 1 ; et des mélanges de ceux-ci.

13. Procédé selon l'une quelconque des revendications 8 à 12 dans lequel le rapport pondéral entre le collecteur primaire et le collecteur secondaire est compris dans la plage de 15:85 à 99:1.
